

## UNITED STATES PATENT OFFICE

2,526,805

## METHOD OF FORMING URANIUM CARBON ALLOYS

James H. Carter, Harrisonburg, Va., and Adrian H. Daane, Ames, Iowa, assignors to the United States of America as represented by the United States Atomic Energy Commission

No Drawing. Application August 12, 1944,  
Serial No. 549,282

2 Claims. (Cl. 75—22)

## 1

This invention relates to uranium-carbon compounds and more particularly to uranium-carbon alloys having a low carbon content. More specifically, our invention is concerned with the formation of uranium carbides and uranium-carbon alloys from uranium metal and carbon.

It is an object of this invention to provide a process for the preparation of uranium-carbon compounds and alloys.

Another object of this invention is to provide a process for the production of uranium-carbon compounds and alloys of low carbon content from uranium and carbon.

A further object of this invention is to provide a process for the production of uranium-carbon compounds and alloys having a selected low carbon content.

Other objects and advantages of this invention will be readily apparent from the following description of preferred embodiments of our invention.

Broadly stated, it has been found that uranium and carbon may be heated in contact with each other at a temperature in excess of the melting point of uranium for a sufficient time to form a desired uranium-carbon compound or alloy.

It has been found that there are two ways of preparing uranium-compounds or alloys in accordance with the method of our invention. One method includes melting uranium metal and placing the molten metal in contact with a carbon surface at a temperature in excess of the melting point of uranium. Carbon is dissolved from the carbon surface by the molten metal, forming a uranium-carbon compound or alloy, and the product obtained upon cooling the solution is substantially homogeneous. Following this method, the uranium is melted and the molten metal is transferred to a carbon crucible, and thereafter the temperature of the crucible and the melt is maintained at the desired temperature for a selected period of time. The amount of carbon dissolved from the carbon surface and, therefore, the composition of the uranium-carbon compound or alloy depend primarily upon the temperature at which the crucible and melt are maintained, and also upon the ratio of carbon surface to the mass of the molten uranium. The composition likewise depends upon the duration of heating and upon the mixing or stirring effected. The uranium-carbon compound formed has a low solubility in the molten uranium metal and during the operation of making the uranium-carbon alloy a carbide crust is formed next to the crucible. Therefore, if the carbon content of the

uranium-carbon alloy produced is to be increased, progressively higher temperatures and stirring during the period of dissolving are required to attain this higher carbon percentage. At low carbon percentages in the uranium-carbon alloy, a slight increase in temperature will produce a relatively large increase in carbon content. However, as the temperature of solution is increased, the additional carbon percentage becomes progressively smaller for each given temperature increment. The desired temperature is maintained for a period of from 20 to 60 minutes. At the end of this time the reaction has taken place between the uranium and carbon and an alloy or compound has been formed. The duration of heating may be such that the increasing carbon content of the uranium-carbon alloy produces an alloy that solidifies at the specific temperature maintained. Uranium-carbon compounds up to at least 9 per cent carbon content and probably with higher carbon content can be produced by this method.

The increase of carbon percentage obtained in the uranium-carbon alloy by the variation in the temperature at which the graphite crucible and melt are maintained is shown by the data in the following table:

Table

| Maximum Temperature<br>°C. | Time at Max. Temp.<br>Minutes | Per Cent in U by weight |
|----------------------------|-------------------------------|-------------------------|
|                            |                               |                         |
| 1,375                      | 40                            | 0.137                   |
| 1,400                      | 20                            | 0.168                   |
| 1,500                      | 60                            | 0.385                   |
| 1,600                      | 20                            | 0.626                   |
| 1,800                      | 30                            | 0.775                   |
| 1,900                      | 30                            | 1.20                    |
| 2,000                      | 30                            | 1.50                    |

Another mode of preparing uranium-carbon compounds or alloys consists in mixing powdered uranium metal with powdered carbon and then pressing the mixture into small blocks under high pressure, 20-50 tons p. s. i., for example, and then heating the pressed blocks in a temperature range above the melting point of uranium and below the melting point of the alloy produced, preferably between 1800° and 2000° C. The operation may be carried on in a graphite or a beryllia crucible. When the process takes place in a graphite crucible, the pressed block is supported on a false bottom of uranium sesquicarbide,  $U_2C_3$ , to prevent the absorption of carbon from the graphite crucible. The heating of the pressed

the sintering of the block causes the uranium carbon alloy to become more compact. The extent to which this sintering or shrinking takes place depends upon the temperature and the period of heating, as the degree of sintering is increased by higher temperatures and longer heating periods. Therefore, the density of the uranium carbon alloy produced is determined among other things by the temperature at which heating is carried on and the length of the period of heating. The temperature is maintained in a range of from 1800° to 2000° C. depending upon the carbon percentage desired in the alloy form. The higher the carbon content the higher the reaction temperature should be maintained. The material is preferably maintained in an atmosphere of carbon dioxide up to the point of the heating of the pressed blocks. The heating is preferably carried on in a vacuum and the temperature during the operation is raised gradually and maintained at the desired maximum for about 10 to 15 minutes.

As an example of the mode of preparing uranium-carbon alloy by the use of pressing and heating carbon and uranium, the mixture consisted of 78.8 grams of powdered uranium and 3 grams of powdered carbon pressed at 20 tons, giving a block  $\frac{1}{2}$  inch x  $\frac{1}{2}$  inch x 2 inches. This block was heated in a zirconia crucible in a vacuum at between 1800° and 2000° C. An analysis of the sample obtained from this process showed a composition of 95.7 per cent uranium by weight and 3.6 per cent carbon, the remaining .7 per cent being unreacted uranium.

It will be apparent to those skilled in the art that various modifications may be made without departing from the principles of the invention as disclosed herein, and for that reason it is not intended that the invention should be limited other than by the scope of the appended claims.

Having thus described our invention, what we claim as novel and desire to secure by Letters Patent of the United States is:

1. The process for forming uranium-carbon alloys consisting of mixing substantially theoretical amounts of powdered uranium and powdered carbon with regard to the final content desired, pressing said mixture and sintering said pressed mixture at a temperature between 1800° C. and 2000° C. in vacuum, whereby said resultant alloy is maintained in the solid state.

2. A process of forming uranium-carbon alloys consisting of mixing uranium powder and carbon powder in the quantities desired in said alloy, compressing the mixture thus produced while maintaining it in an atmosphere of carbon dioxide, and heating said compressed product to a temperature ranging from 1800° to 2000° C., whereby said resultant alloy is maintained in the solid state.

JAMES H. CARTER.  
ADRIAN H. DAANE.

#### REFERENCES CITED

The following references are of record in the file of this patent:

#### UNITED STATES PATENTS

| Number    | Name        | Date          |
|-----------|-------------|---------------|
| 1,829,950 | Voigtlander | Nov. 3, 1931  |
| 1,876,175 | Stoody      | Sept. 6, 1932 |
| 2,113,171 | Cooper      | Apr. 5, 1938  |

#### OTHER REFERENCES

Lohman: Article in *Elektrochem. z.*, 26, 29-33 (1919); briefed in *Chemical Abstracts*, vol. 14, 1920, page 1081.

Mellor: "Comprehensive Treatise on Inorganic and Theoretical Chemistry," vol. 12, 1932, pages 10, 11; and vol. 5, 1932, page 890.

Hopkins: "Chapters in the Chemistry of the Less Familiar Elements," vol. II, chapter 18, 1940, pages 6 and 14-16.